

# United States Patent Office

3,336,168

Patented Aug. 15, 1967

1

3,336,168

WELDABLE TOUGH STEEL ESSENTIALLY COMPOSED OF CHROMIUM AND MANGANESE AND METHOD OF MANUFACTURING THE SAME  
Sadayoshi Morita, Susumu Goda, Makoto Sato, and Yoshinori Yamaguchi, all of Kitakyushu, Fukuoka Prefecture, Japan, assignors to Yawata Iron & Steel Co., Ltd., Tokyo, Japan

No Drawing. Continuation of application Ser. No. 319,504, Oct. 28, 1963. This application Dec. 30, 1966, Ser. No. 606,447

Claims priority, application Japan, Nov. 1, 1962, 37/49,242

1 Claim. (Cl. 148—38)

This is a continuation of application Ser. No. 319,504, filed Oct. 28, 1963, now abandoned.

This invention relates to a tough steel of good weldability, and more particularly relates to a super high tension steel essentially composed of chromium and manganese, in which nickel is contained in much smaller amount than that in any conventional high tension steel.

As a conventional super high tension steel there may be enumerated such kinds of steels as SAE 4340 type steel, hot-rolled die-steel, cold-rolled AISI type 301 series steel or PH stainless steel. Among them PH stainless steel is most frequently used because of its superior qualities in weldability, workability and anticorrosiveness. However, it has a defect in relatively high production cost, because it contains a relatively high percentage of nickel.

As a result of investigations the inventors have discovered that a tough steel of novel composition series, in which nickel is reduced to an amount less than 3.5 wt. percent and chromium and manganese are the essential constituents in place thereof, renders such a superior weld as never found in the conventional high tension steels.

The main object of the present invention is to provide a novel tough steel characterized by a good weldability even with a lower nickel content than that in any conventional tough steel.

Another object of the present invention is to provide a novel weldable steel of superior qualities at much lower production cost than that of any conventional tough steel.

Further objects of the present invention is to provide a weldable tough steel of a novel composition series, in which nickel is contained in an amount less than 3.5 wt. percent and chromium and manganese are the essential constituents.

Further objects of the present invention is to provide a method of manufacturing the aforesaid weldable tough steel of a novel composition series.

According to the method of the present invention three series of weldable tough steels essentially composed of chromium and manganese may be obtained, that is,

(1) The weldable tough steel of the first series is characterized by the following composition:

|    |                |
|----|----------------|
| C  | Wt. percent    |
| Si | Less than 0.20 |
| Cr | Less than 1.5  |
|    | 3.0 to 17.0    |

2

Wt. percent

|    |               |
|----|---------------|
| Ni | Less than 3.5 |
| Mn | 2.0 to 10.0   |
| Cu | 0.2 to 5.0    |

5 Balance accompanying impurities and iron.

(2) The weldable tough steel of the second series is characterized by the following composition:

Wt. percent

|    |                |
|----|----------------|
| C  | Less than 0.20 |
| Si | 0.08 to 1.0    |
| Cr | 3.0 to 17.0    |
| Ni | 0.1 to 3.5     |
| Mn | 3.5 to 10.0    |
| Cu | 0.2 to 5.0     |
| Mo | 0.3 to 3.0     |
| Al | 0.003 to 1.0   |

Balance accompanying impurities and iron.

Besides the aforesaid alloying elements this series of the weldable tough steel may contain the following elements according to the necessities:

One or more than two kinds of elements selected from a group consisting of V, Nb, Ta and

|    |                                              |
|----|----------------------------------------------|
| Ti | 0 to 10 times so much as C content in total. |
| N  | 0 to 0.2 wt. percent.                        |
| Be | 0 to 0.25 wt. percent.                       |

30 in which 0 designates no addition.

The last second series tough steel differs from the first series in that besides C, Si, Cr, Ni, Mn and Cu there are added Mo, Al, N, Be and one or more than two kinds of elements selected from a group consisting of V, Nb, Ta and Ti.

(3) The third series of weldable tough steel is characterized by the following composition:

|    |                             |
|----|-----------------------------|
| C  | Less than 0.20 wt. percent. |
| Si | Less than 1.5 wt. percent.  |
| Cr | 3.0 to 17.0 wt. percent.    |

|    |                            |
|----|----------------------------|
| Ni | Less than 3.5 wt. percent. |
| Mn | 2.0 to 10.0 wt. percent.   |
| Cu | 0.2 to 5.0 wt. percent.    |

|                |                                  |
|----------------|----------------------------------|
| 45 Mo or/and W | 0.4 to 3.0 wt. percent in total. |
|----------------|----------------------------------|

N Less than 0.2 wt. percent.

One or more than two kinds of elements selected from a group consisting of V, Nb, Ta Ti and Al Less than 1.5 wt. percent in total.

55 The difference between the second and third series resides in that in the latter W is added in place of or together with Mo.

By elucidating the criticality of each element in the compositions of the aforesaid weldable tough steels the features of the present invention will be made clear.

60 In general, the carbon content of steel is desirable to be low to improve the weldability thereof and the percentage of less than 0.20 was found to be adequate to maintain the weldability and notch toughness. Si serves to re-

markedly improve the acid-resistance of steel when it co-exists with Cr. By adding Si up to 1.5 wt. percent to steel a favorable result could be obtained. If more than 1.5 wt. percent, the toughness of steel was sacrificed. Cr improves the anticorrosiveness, lowers the Ms temperature and is necessary to obtain the desired structure of steel. By adding Cr in the range of 3 to 17.0 wt. percent to steel the expected results were obtained. Less than 3 wt. percent, no effect of the addition of this element was demonstrated and more than 17 wt. percent, the  $\delta$  ferrite was precipitated, thereby the strength of steel was damaged. As the present invention is to improve the weldability by leaving some quantity of the austenite in the weld, it is necessary to confine the amount of  $\delta$  ferrite to be produced by the addition of Cr to a proper amount. For this purpose the addition of the austenite-forming elements such as C, Ni, Mn and N in proper amounts are required to counterbalance the effects of the ferrite-forming elements such as Cr, Si, Mo and the like. As Ni is limited to a relatively low amount in the steel prepared by the present invention, the content of Mn is to be regulated to obtain the desired structure of steel. The addition of Mn in an amount of 2.0 to 10.0 wt. percent, preferably 3.0 to 8.0 wt. percent, was found to be adequate. A higher amount than 10.0 wt. percent produces stable austenite, thereby the hardening is hampered. Further, the amount of Ni should be reduced in correspondence with Cr in order to prevent the formation of  $\delta$  ferrite. However, in view of the necessity of preserving the anticorrosiveness of steel the lower limit of the addition of Ni should be such as to balance with 10 wt. percent of Cr to be added.

Cu serves to stabilize the austenite and provide steel with the precipitation hardenability by itself or the compounds made by the reaction with afterwards mentioned precipitation-hardening elements. Cu was proved to be a cheap and effective strength-increasing element. For this reason Cu was added up to about 5 wt. percent in the steel prepared by the present invention. However, a higher percentage than that causes remarkable red shortness. The lower limit thereof was 0.2 wt. percent. Below this lower limit, there appeared no precipitation effect. But, when it co-exists with V, Nb and Ti and the like, the precipitation hardenability increases by the synergistical effect, thereby the required addition of Cu may be reduced.

Besides the aforesaid C, Si, Cr, Mn and Cu, there were further added 0.003 to 1.0 wt. percent of Al, 0 to 10 times so much as C content of one or more than two kinds of elements selected from the group consisting of V, Nb, Ta and Ti, and 0 to 0.2 wt. percent of N and 0 to 0.25 wt. percent of Be in the tough steel of the second series prepared by the present invention. V, Nb, Ta and Ti function as precipitation-hardening elements. These elements produce intermetallic compounds in combination with Mn, Cu and Ni, which compounds effect the precipitation-hardening in the martensitic structure formed by the tempering, thereby the yield strength of steel is enhanced. That is, by the addition of these elements a steel superior in hot-workability and weldability may be obtained due to a favorable precipitation-hardenability given by them. Al and Be belong also to the precipitation-hardening elements. Further, Al is required to effect the grain-refining. The addition of Al up to 1.0 wt. percent was effective, but below 0.003 wt. percent no effect could be perceived. Be could be added up to 0.25 wt. percent. The addition of N up to 0.2 wt. percent was possible when no nitride-forming element such as V, Nb, Ta and Ti was added, but when the nitride-forming element was added, the addition of N of below 0.12 wt. percent was adequate, particularly below 0.05 wt. percent.

As already mentioned, the weldable tough steel of the third series is distinguished from that of the second series by the addition of W in place of or together with Mo.

W and Mo have the effects of preventing the temper brittleness, improving the low-temperature toughness and increasing the temper resistance by the secondary hardening effected at the time of tempering. In view of the economic conditions the addition of both elements or of one of them up to 3 wt. percent was feasible, but no effect could be perceived with an addition of below 0.4 wt. percent.

Summarily, the compositions of the aforesaid tough steels prepared by the present invention may be characterized by the following three features: Ni is substituted by Cr and Mn to economize the former, various kinds of precipitation-hardening elements, particularly those of the group consisting of V, Nb, Ta and Ti, are used to improve the weldability and hot-workability, and W is used as an equivalent of Mo for preventing the temper brittleness and improving the temper resistance.

The method of manufacturing the weldable tough steel according to the present invention has somewhat different steps according to the series of compositions, though in principle the same. In the case of the second series of composition, after the specified elements have been added to a steel containing less than 0.20 wt. percent of C to prepare an alloyed steel, said alloyed steel is hot-rolled, then the hot-rolled steel is subjected to a solution treatment, the steel is held at a temperature of  $Ac_3$  to 1,100° C. for 1-3 hours and then subjected to an air-cooling. The solution treatment may be carried out more than one time. The solution treatment is immediately followed by the tempering treatment at a temperature of below  $Ac_1$  to effect the precipitation-hardening. It is also possible to carry out between the solution treatment and tempering treatment a sub-zero treatment, in which the steel is held at a temperature below zero degree for 2 to 3 hours to develop the transformation from austenite to martensite, or a martensitic transformation from austenite to martensite by reheating the material up to the temperature above  $Ac_3$  transformation point. That is, the tempering process may be carried out after the martensitic transformation has been effected.

Also in the case of the third series of the composition, after the specified elements have been added to a steel containing less than 0.20 wt. percent of C to prepare an alloyed steel, said alloyed steel is subjected to the same heat treatments as above mentioned. However, in this case, the heat treatment comprises only the steps of the solution treatment and tempering treatment, when the sum of Ni content and  $\frac{1}{2}$  Mn content amounts to about 3 to 5 wt. percent, and when the sum of Ni content and  $\frac{1}{2}$  Mn content exceeds about 5 wt. percent, the step of the martensitic transformation treatment or cold-rolling or sub-zero treatment is interposed between the solution treatment and the tempering treatment, because in the former case, that is, in the case of the sum of Ni and  $\frac{1}{2}$  Mn amounting to about 3 to 5 wt. percent only a small amount of austenite remains in the martensitic structure after the solution treatment has been carried out and hence the desired product may be obtained by immediately carrying out the sequent precipitation-hardening treatment, whereas as in the latter case, that is, in the case of the sum of both elements exceeding about 5 wt. percent a large amount of austenite still remains in the martensitic structure after the solution treatment it is necessary to carry out the intermediate treatment such as the martensitic transformation treatment or cold-rolling or sub-zero treatment to produce the martensitic structure before the precipitation-hardening treatment is carried out.

#### Example 1

Tests have been carried out on four specimens of the second series of the composition as shown in Table 1.

TABLE 1.—CHEMICAL COMPOSITION IN WEIGHT PERCENT

| Steel specimen | C    | Si   | Mn   | Ni   | Cr   | Mo   | Cu   | Ti    | Nb    | V     | Al    | N     |
|----------------|------|------|------|------|------|------|------|-------|-------|-------|-------|-------|
| A-----         | 0.08 | 0.31 | 5.2  | 0.8  | 6.91 | 0.54 | 0.72 | ----- | ----- | ----- | 0.032 | ----- |
| B-----         | 0.11 | 0.33 | 5.3  | 0.7  | 12.1 | 1.5  | 0.91 | ----- | ----- | ----- | 0.051 | ----- |
| C-----         | 0.12 | 0.23 | 5.20 | 1.95 | 6.92 | 1.50 | 0.87 | 0.21  | 0.07  | ----- | 0.027 | ----- |
| D-----         | 0.11 | 0.33 | 7.80 | 1.83 | 12.0 | 0.56 | 1.00 | ----- | ----- | ----- | 0.25  | 0.11  |

After the specified alloying elements have been added to a steel containing less than 0.20 wt. percent of C, the

400 Hv (Vickers hardness), indicating that the welding hardening occurred in a small degree.

TABLE 2.—MECHANICAL PROPERTIES

| Steel specimen | Thickness of steel (mm.) | Heat treatment                          |                            |                                          | 0.2% elongation proof stress (kg./mm. <sup>2</sup> ) | Tensile strength (kg./mm. <sup>2</sup> ) | Elongation GL 50 mm. (percent) | 0° C. V Charpy impact value (kg.-m./cm. <sup>2</sup> ) | Hardness of weld accord to thermocycle reproduction method (Hv) |
|----------------|--------------------------|-----------------------------------------|----------------------------|------------------------------------------|------------------------------------------------------|------------------------------------------|--------------------------------|--------------------------------------------------------|-----------------------------------------------------------------|
|                |                          | Primary tr. (solution treatment) (° C.) | Secondary treatment (° C.) | Precipitation hardening treatment (° C.) |                                                      |                                          |                                |                                                        |                                                                 |
| A-----         | 20                       | 1,050                                   | -----                      | 450                                      | 104                                                  | 131                                      | 17.0                           | 4.9                                                    | 406                                                             |
|                |                          | 950                                     | -----                      | 450                                      | 106                                                  | 127                                      | 15.5                           | 4.6                                                    | 403                                                             |
| B-----         | 20                       | 1,050                                   | 400                        | 400                                      | 108                                                  | 139                                      | 16.4                           | 5.3                                                    | 435                                                             |
|                |                          | 950                                     | 400                        | 400                                      | 110                                                  | 141                                      | 16.2                           | 4.5                                                    | 432                                                             |
| C-----         | 20                       | 1,050                                   | 400                        | 400                                      | 111                                                  | 135                                      | 18.0                           | 6.0                                                    | -----                                                           |
|                |                          | 950                                     | 400                        | 400                                      | 112                                                  | 136                                      | 17.0                           | 6.4                                                    | 430                                                             |
| D-----         | 25                       | 1,050                                   | *750                       | 500                                      | 105                                                  | 127                                      | 15.0                           | 4.4                                                    | 370                                                             |
|                |                          | -----                                   | -----                      | 500                                      | 103                                                  | 125                                      | 16.5                           | 5.3                                                    | 375                                                             |

\* Transformation treatment.

alloyed steels were rolled to 20 and 25 mm. in thickness and then

(a) The specimen A of 20 mm. in thickness was normalized at temperatures of 1,050° C. and 950° C. (solution treatment) and then tempered at a temperature of 450° C. (precipitation treatment).

### Example 2

35 Tests have been carried out on five specimens of the third series of the composition, as shown in Table 3. The hot-rolled specimens were subjected to the following heat treatments:

TABLE 3.—CHEMICAL COMPOSITION IN WEIGHT PERCENT

| Steel specimen | C    | Si   | Mn   | P     | S     | Ni   | Cr   | Mo   | W     | Cu   | Ti   | Nb    | V     | Ta    | N     | O     | Al |
|----------------|------|------|------|-------|-------|------|------|------|-------|------|------|-------|-------|-------|-------|-------|----|
| 1-----         | 0.09 | 0.21 | 4.40 | 0.018 | 0.023 | 2.10 | 12.3 | 1.60 | ----- | 2.20 | 0.14 | ----- | ----- | ----- | 0.012 | 0.060 |    |
| 2-----         | 0.07 | 0.19 | 4.20 | 0.021 | 0.025 | 2.20 | 12.0 | 1.52 | 0.20  | 2.43 | 0.18 | ----- | ----- | 0.08  | 0.010 | 0.075 |    |
| 3-----         | 0.06 | 0.25 | 4.53 | 0.019 | 0.023 | 2.10 | 13.8 | 1.33 | 0.55  | 2.10 | 0.15 | 0.05  | 0.02  | 0.02  | 0.012 | 0.075 |    |
| 4-----         | 0.08 | 0.23 | 7.40 | 0.018 | 0.020 | 2.05 | 14.0 | 1.35 | 0.50  | 2.21 | 0.10 | 0.02  | 0.02  | 0.02  | 0.015 | 0.071 |    |
| 5-----         | 0.10 | 0.24 | 7.50 | 0.020 | 0.025 | 2.15 | 14.1 | 1.65 | ----- | 2.15 | 0.13 | 0.04  | 0.04  | 0.04  | 0.016 | 0.085 |    |

(b) The specimen B of 20 mm. in thickness was normalized at temperatures of 1,050° C. and 950° C. and then tempered at a temperature of 400° C.,

(c) The specimen C of 20 mm. in thickness was normalized at temperatures of 1,050° C. and 950° C. and then tempered at a temperature of 400° C.,

(d) The specimen D of 25 mm. in thickness was normalized at a temperature of 1,050° C. and then subjected to transformation treatment at a temperature of 750° C. and subsequently was tempered at a temperature of 500° C.

Another sample of D was only tempered at a temperature of 500° C. without carrying out the normalizing process (solution treatment).

The results obtained by these processes are shown in Table 2. As evidently seen from Table 2, in all specimens a tensile strength above 120 kg./mm.<sup>2</sup> could be achieved. The V Charpy impact test at 0° C. showed 4.4 to 7.9 kg.-m./cm.<sup>2</sup>, demonstrating the sufficient toughness required for the high tension steel of this kind. Further, the test of the highest hardness of weld according to the welding thermocycle reproduction method showed around

55 (a) The specimens 1, 2 and 3 of 12 mm. in thickness were subjected to the solution treatment at a temperature of 1,050° C. and then tempered at a temperature of 460° C. (precipitation treatment) (martensite type steel plate),

60 (b) The specimens 4 and 5 of 12 mm. in thickness were subjected to the solution treatment at a temperature of 950° C. and then to the transformation treatment at a temperature of 750° C. and subsequently to the precipitation treatment at a temperature of 460° C. (semi-austenite type steel plate).

65 Another sample of 4 and 5 of 3 mm. in thickness were subjected to the solution treatment at a temperature of 1,050° C. and then to the cold-rolling and the cold-rolled materials were subjected to the precipitation treatment at a temperature of 460° C.

70 Further samples of 4 and 5 of 12 mm. in thickness were subjected to the solution treatment at a temperature of 950° C., then to the sub-zero treatment at a temperature of -70 to -80° C. with a holding time of 2 to 3 hours and then subsequently to the precipitation treatment at a temperature of 460° C.

The results obtained by these processes are shown in Table 4. Also in these cases, a yield strength of above 120 kg./mm.<sup>2</sup> and an elongation (gauge length 50 mm.) of 8 to 15% were obtained, indicating the strength and ductility sufficiently comparable with Ni-Cr type precipi-

5 tation-hardened stainless steel. wt. percent Si, 3.0 to 17.0 wt. percent Cr, less than 3.5 wt. percent Ni, 2.0 to 10.0 wt. percent Mn, 0.2 to 5.0 wt. percent Cu, 0.003 to 1.0 wt. percent Al, 0.3 to 3.0 wt. percent of an element selected from the group consisting of Mo and W, an element selected from the group consisting of V, Nb, Ta and Ti in an amount less than

TABLE 4.—MECHANICAL PROPERTIES

| Steel specimen | Thickness of steel (mm.) | Heat treatment                 |                                             |                                             | $\sigma_y$ 0.2% elongation proof stress (kg./mm. <sup>2</sup> ) | $\sigma_B$ (kg./mm. <sup>2</sup> ) | Elongation GL 50 mm. (percent) |
|----------------|--------------------------|--------------------------------|---------------------------------------------|---------------------------------------------|-----------------------------------------------------------------|------------------------------------|--------------------------------|
|                |                          | Primary treatment              | Secondary treatment                         | Third treatment                             |                                                                 |                                    |                                |
| 1-----         | 12                       | Solution treatment at 1,050° C | Precipitation hardening treatment at 460° C | -----                                       | 127                                                             | 139                                | 10                             |
| 2-----         | 12                       | do                             | do                                          | -----                                       | 125                                                             | 143                                | 11                             |
| 3-----         | 12                       | do                             | Transformation treatment at 750° C          | Precipitation hardening treatment at 460° C | 128                                                             | 142                                | 10                             |
| 4-----         | 3                        | Solution treatment at 1,050° C | Cold rolling                                | do                                          | 130                                                             | 145                                | 9                              |
| 4-----         | 12                       | Solution treatment at 950° C   | Sub-zero treatment                          | do                                          | 145                                                             | 161                                | 8                              |
| 5-----         | 12                       | Solution treatment at 950° C   | Transformation treatment at 750° C          | do                                          | 126                                                             | 147                                | 12                             |
| 5-----         | 3                        | Solution treatment at 1,050° C | Cold-rolling                                | do                                          | 128                                                             | 146                                | 8                              |
| 5-----         | 12                       | Solution treatment at 950° C   | Sub-zero treatment                          | do                                          | 148                                                             | 165                                | 9                              |
|                |                          |                                |                                             | do                                          | 130                                                             | 148                                | 11                             |

What is claimed is:

A weldable tough steel obtained by subjecting a steel consisting of less than 0.2 wt. percent C, less than 1.5

10 times so much as the C content and the rest being iron and impurities, to the precipitation-hardening treatment.

#### References Cited

##### UNITED STATES PATENTS

- |           |         |               |       |            |
|-----------|---------|---------------|-------|------------|
| 2,198,598 | 4/1940  | Becket et al. | ----- | 75—126     |
| 2,948,603 | 8/1960  | Pitler et al. | ----- | 148—38 X   |
| 3,152,934 | 10/1964 | Lula et al.   | ----- | 148—12.3 X |

##### FOREIGN PATENTS

- 832,562 4/1960 Great Britain.

DAVID L. RECK, *Primary Examiner.*